



US007491443B2

(12) **United States Patent**  
**Mackey et al.**

(10) **Patent No.:** **US 7,491,443 B2**  
(b4) **Date of Patent:** **Feb. 17, 2009**

(54) **POLYSACCHARIDE STRUCTURES  
COMPRISING AN UNSUBSTITUTED  
POLYSACCHARIDE AND PROCESSES FOR  
MAKING SAME**

(75) Inventors: **Larry Neil Mackey**, Fairfield, OH (US);  
**Gregory Charles Gordon**, Cincinnati, OH (US); **Stephen Wayne Heinzman**, Cincinnati, OH (US)

(73) Assignee: **The Procter & Gamble Company**, Cincinnati, OH (US)

(\*) Notice: Subject to any disclaimer, the term of this patent is extended or adjusted under 35 U.S.C. 154(b) by 0 days.

(21) Appl. No.: **12/118,784**

(22) Filed: **May 12, 2008**

(65) **Prior Publication Data**

US 2008/0213586 A1 Sep. 4, 2008

**Related U.S. Application Data**

(60) Division of application No. 11/296,629, filed on Dec. 7, 2005, now Pat. No. 7,390,565, which is a continuation-in-part of application No. 11/018,746, filed on Dec. 20, 2004, now abandoned.

(51) **Int. Cl.**  
**D02G 3/00** (2006.01)

(52) **U.S. Cl.** ..... 428/372; 428/364; 428/393

(58) **Field of Classification Search** ..... 428/364, 428/372, 393, 394; 536/30

See application file for complete search history.

(56) **References Cited**

**U.S. PATENT DOCUMENTS**

6,551,705 B1 \* 4/2003 Ohnishi et al. ..... 428/372  
6,709,526 B1 3/2004 Bailey et al.

|                   |         |                               |
|-------------------|---------|-------------------------------|
| 6,723,160 B2      | 4/2004  | Mackey et al.                 |
| 6,802,895 B2      | 10/2004 | Mackey et al.                 |
| 6,811,740 B2      | 11/2004 | James et al.                  |
| 6,955,850 B1      | 10/2005 | Cabell et al.                 |
| 6,977,116 B2      | 12/2005 | Cabell et al.                 |
| 7,041,369 B1      | 5/2006  | Mackey et al.                 |
| 7,229,689 B2 *    | 6/2007  | Qin et al. ..... 428/372      |
| 7,276,201 B2      | 10/2007 | James et al.                  |
| 7,390,565 B2 *    | 6/2008  | Mackey et al. ..... 428/364   |
| 2003/0201579 A1   | 10/2003 | Gordon et al.                 |
| 2003/0203196 A1   | 10/2003 | Trokhman et al.               |
| 2004/0132873 A1   | 7/2004  | Bailey et al.                 |
| 2004/0249066 A1   | 12/2004 | Heinzman et al.               |
| 2005/0076809 A1 * | 4/2005  | Mackey et al. ..... 106/206.1 |
| 2005/0136253 A1   | 6/2005  | Michael et al.                |
| 2005/0137330 A1   | 6/2005  | Forshey et al.                |
| 2005/0137331 A1   | 6/2005  | Forshey et al.                |
| 2005/0263938 A1   | 12/2005 | Cabell et al.                 |
| 2005/0275133 A1   | 12/2005 | Cabell et al.                 |
| 2005/0279470 A1   | 12/2005 | Redd et al.                   |
| 2005/0281978 A1   | 12/2005 | Cabell et al.                 |
| 2006/0134045 A1 * | 6/2006  | Cao et al. ..... 424/70.13    |
| 2006/0134410 A1 * | 6/2006  | Mackey et al. ..... 428/364   |
| 2006/0134411 A1 * | 6/2006  | Mackey et al. ..... 428/364   |
| 2006/0134412 A1 * | 6/2006  | Mackey et al. ..... 428/364   |
| 2006/0275347 A1   | 12/2006 | Evers Smith et al.            |
| 2006/0287519 A1   | 12/2006 | Heinzman                      |
| 2008/0213586 A1 * | 9/2008  | Mackey et al. ..... 428/364   |

**OTHER PUBLICATIONS**

U.S Appl. No. 09/914,966, filed Mar. 8, 1999, Mackey et al.

\* cited by examiner

*Primary Examiner*—N. Edwards

(74) *Attorney, Agent, or Firm*—C. Brant Cook

(57) **ABSTRACT**

Polysaccharides, more particularly, polysaccharide structures, especially fibers, comprising an unsubstituted polysaccharide, webs comprising such polysaccharide structures and processes for making such polysaccharide structures and/or webs are provided.

**13 Claims, 4 Drawing Sheets**





Fig. 1A



Fig. 1B



Fig. 2



Fig. 3



Fig. 4



Fig. 5

Fig. 6



## 1

**POLYSACCHARIDE STRUCTURES  
COMPRISING AN UNSUBSTITUTED  
POLYSACCHARIDE AND PROCESSES FOR  
MAKING SAME**

**CROSS REFERENCE TO RELATED  
APPLICATION**

The present application is a divisional application of U.S. application Ser. No. 11/296,629 filed Dec. 7, 2005 now U.S. Pat. No. 7,390,565, which is a continuation-in-part application of U.S. application Ser. No. 11/018,746 filed Dec. 20, 2004 now abandoned.

**FIELD OF THE INVENTION**

The present invention relates to polysaccharides, more particularly, to polysaccharide structures, especially fibers, comprising an unsubstituted polysaccharide, webs comprising such polysaccharide structures and processes for making such polysaccharide structures and/or webs.

**BACKGROUND OF THE INVENTION**

Polysaccharide structures, such as fibers and/or films, comprising polysaccharides are known in the art. However, polysaccharide structures, especially in the form of fibers, comprising unsubstituted polysaccharides wherein the polysaccharide structures exhibit an apparent peak wet tensile stress greater than 0.2 MPa and/or an average fiber diameter of less than 10  $\mu\text{m}$  have been until now unobtainable.

Accordingly, there exists a need for polysaccharide structures that comprise unsubstituted polysaccharides wherein the polysaccharide structures exhibit an apparent peak wet tensile stress greater than 0.2 MPa and/or an average fiber diameter of less than 10  $\mu\text{m}$ , webs comprising such polysaccharide structures and processes for making such polysaccharide structures.

**SUMMARY OF THE INVENTION**

The present invention fulfills the needs described above by providing polysaccharide structures comprising an unsubstituted polysaccharides and/or webs comprising such polysaccharide structures and processes for making such polysaccharide structures and/or webs.

In one example of the present invention, a polysaccharide structure, such as a fiber, comprising an unsubstituted polysaccharide wherein the polysaccharide structure exhibits an apparent peak wet tensile stress greater than 0.2 MPa is provided.

In another example of the present invention, a fiber comprising an unsubstituted polysaccharide wherein the fiber exhibits an average fiber diameter of less than 10  $\mu\text{m}$  is provided.

In another example of the present invention, a web comprising a polysaccharide structure according to the present invention is provided.

In yet another example of the present invention, a process for making a polysaccharide structure comprising an unsubstituted polysaccharide, wherein the process comprises the step of processing a polysaccharide-containing composition comprising a substituted polysaccharide into a polysaccharide structure comprising an unsubstituted form of the substituted polysaccharide, is provided.

In still another example of the present invention, a process for making a polysaccharide structure comprising an unsub-

## 2

stituted polysaccharide, wherein the process comprises the step of processing a polysaccharide-containing composition comprising an unsubstituted polysaccharide into a polysaccharide structure comprising the unsubstituted polysaccharide, is provided.

In even yet another example of the present invention, a process for making a polysaccharide structure comprising an unsubstituted polysaccharide, wherein the process comprises the steps of:

- 10 a. providing a polysaccharide-containing composition comprising an unsubstituted polysaccharide;
- b. substituting the unsubstituted polysaccharide to produce a substituted polysaccharide; and
- 15 c. processing the polysaccharide-containing composition comprising the substituted polysaccharide into a polysaccharide structure comprising the unsubstituted polysaccharide, is provided.

Accordingly, the present invention provides a polysaccharide structure comprising an unsubstituted polysaccharide, a web comprising such a polysaccharide structure and a process for making such a polysaccharide structure and/or web.

**BRIEF DESCRIPTION OF THE DRAWINGS**

FIG. 1A is a schematic side view of a barrel of a twin screw extruder suitable for use in the present invention.

FIG. 1B is a schematic side view of a screw and mixing element configuration suitable for use in the barrel of FIG. 1A.

FIG. 2 is a schematic side view of a process for synthesizing a polysaccharide structure in accordance with the present invention.

FIG. 3 is a schematic partial side view of the process of the present invention, showing an attenuation zone.

FIG. 4 is a schematic plan view taken along lines 4-4 of FIG. 3 and showing one possible arrangement of a plurality of extrusion nozzles arranged to provide polysaccharide structures of the present invention.

FIG. 5 is a view similar to that of FIG. 4 and showing one possible arrangement of orifices for providing a boundary air around the attenuation zone.

FIG. 6 is a schematic plan view of a coupon that can be used for determining apparent peak wet tensile stress of fibers according to the present invention.

**DETAILED DESCRIPTION OF THE INVENTION**

**Definitions**

“Polysaccharide structure” as used herein means any physical structure formed as a result of processing a polysaccharide-containing composition into such a physical structure. Nonlimiting examples of polysaccharide structures in accordance with the present invention include fibers, films and/or foams. The polysaccharide structures of the present invention are non-naturally occurring physical structures. In other words, they are man-made physical structures.

“Fiber” or “filament” as used herein means a slender, thin, and highly flexible object having a major axis which is very long, compared to the fiber’s two mutually-orthogonal axes that are perpendicular to the major axis. A fiber may exhibit an aspect ratio of the major’s axis length to an equivalent diameter of the fiber’s cross-section perpendicular to the major axis is greater than 100/1, more specifically greater than 500/1, and still more specifically greater than 1000/1, and

even more specifically, greater than 5000/1. The fibers may be continuous or substantially continuous fibers or they may be discontinuous fibers.

The fibers comprising an unsubstituted polysaccharide of the present invention may have an average fiber diameter of less than about 50  $\mu\text{m}$  and/or less than about 20  $\mu\text{m}$  and/or less than about 10  $\mu\text{m}$  and/or less than about 8  $\mu\text{m}$  and/or less than about 6  $\mu\text{m}$  and/or less than about 4  $\mu\text{m}$  as measured by the Average Fiber Diameter Test Method described herein. Such a fiber may exhibit an average fiber diameter of greater than about 1  $\mu\text{m}$  and/or greater than about 2  $\mu\text{m}$  and/or greater than about 3  $\mu\text{m}$ .

The fibers comprising an unsubstituted polysaccharide of the present invention may include melt blown fibers, dry spun fibers, rotary spun fibers, spunbond fibers, staple fibers, hollow fibers, shaped fibers, such as multi-lobal fibers and multicomponent fibers, especially bicomponent fibers. The multicomponent fibers, especially bicomponent fibers, may be in a side-by-side, sheath-core, segmented pie, ribbon, islands-in-the-sea configuration, or any combination thereof. The sheath may be continuous or non-continuous around the core. The ratio of the weight of the sheath to the core can be from about 5:95 to about 95:5. The fibers comprising an unsubstituted polysaccharide of the present invention may have different geometries that include round, elliptical, star shaped, rectangular, and other various eccentricities.

In another example, the polysaccharide structures of the present invention may include a multiconstituent polysaccharide structure, such as a multicomponent fiber, comprising an unsubstituted polysaccharide of the present invention along with a polymer. A multicomponent fiber, as used herein, means a fiber having more than one separate part in spatial relationship to one another. Multicomponent fibers include bicomponent fibers, which is defined as a fiber having two separate parts in a spatial relationship to one another. The different components of multicomponent fibers can be arranged in substantially distinct regions across the cross-section of the fiber and extend continuously along the length of the fiber.

A nonlimiting example of such a multicomponent fiber, specifically a bicomponent fiber, is a bicomponent fiber in which the unsubstituted polysaccharide of the present invention represents the core of the fiber and a polymer represents the sheath, which surrounds or substantially surrounds the core of the fiber. The polysaccharide-containing composition from which such a polysaccharide structure is derived may include both the polysaccharide and the other polymer.

In another multicomponent, especially bicomponent fiber embodiment, the sheath may comprise a polysaccharide and a crosslinking system having a crosslinking agent, and the core may comprise a polysaccharide and a crosslinking system having a crosslinking agent. With respect to the sheath and core, the polysaccharide may be the same or different and the crosslinking agent may be the same or different. Further, the level of polysaccharide may be the same or different and the level of crosslinking agent may be the same or different.

One or more polysaccharide structures of the present invention may be incorporated into a multi-polysaccharide structure product, such as a fibrous structure and/or web, if the polysaccharide structures are in the form of fibers. Such a multi-polysaccharide structure product may ultimately be incorporated into a commercial product, such as a single- or multi-ply sanitary tissue product, such as facial tissue, bath tissue, paper towels and/or wipes, feminine care products, diapers, writing papers, cores, such as tissue cores, and other types of paper products.

“Web” as used herein means a fibrous structure and/or a film. In one example, a web is a physical structure that comprises at least one planar surface. In another example, a web is a physical structure that comprises two planar surfaces.

5 One or more fibers at least one of which is a fiber comprising an unsubstituted polysaccharide of the present invention may be associated to form a web. Typically, numerous fibers are collected, such as on a forming wire or belt, in order to associate the fibers into a web.

10 In one example of the present invention, a web of the present invention exhibits an initial total wet tensile of greater than about 10 g/2.54 cm (10 g/in).

“Hydroxyl polymer” as used herein means any polymer that contains greater than 10% and/or greater than 20% and/or 15 greater than 25% by weight hydroxyl groups.

“Polysaccharide-containing composition” as used herein means a composition that comprises a polysaccharide (substituted or unsubstituted).

“Unsubstituted polysaccharide” and/or “unsubstituted 20 form of a polysaccharide” and/or “unsubstituted form of a substituted polysaccharide” as used herein means a polysaccharide in which all of its free (not part of a crosslink) hydroxyl moieties are intact. In other words, no free (not part of a crosslink) derivatized hydroxyl moieties exist in the 25 polysaccharide. For purposes of the present invention, the mere removal of the hydrogen from the oxygen in the hydroxyl moieties does not create a substituted polysaccharide.

“Substituted polysaccharide” and/or “substituted form of a 30 polysaccharide” and/or “substituted form of an unsubstituted polysaccharide” as used herein means a polysaccharide comprising at least one derivatized hydroxyl moiety. In other words, at least one oxygen originally present in a hydroxyl moiety is covalently bonded to a moiety other than hydrogen. 35 Original hydroxyl moieties that have form crosslinks are not, for purposes of the present invention, “substituted.”

“Unsubstituted polysaccharide-containing composition” as used herein means a composition that comprises at least one unsubstituted polysaccharide. In one example, the unsubstituted 40 polysaccharide-containing composition comprises at least one material that doesn’t melt before it decomposes. For example, an unsubstituted polysaccharide can dissolve and/or be plasticized in water, rather than melt in the absence of a plasticizer, and then can be dried (removal of water) during a 45 polysaccharide structure forming process.

“Apparent Peak Wet Tensile Stress,” or simply “Wet Tensile Stress,” is a condition existing within a polysaccharide structure, such as a fiber, at the point of its maximum (i.e., “peak”) stress as a result of strain by external forces, and more 50 specifically elongation forces, as described in the Apparent Peak Wet Tensile Stress Test Method described herein below. The stress is “apparent” because a change, if any, in the polysaccharide structures average thickness, such as a fiber’s average fiber diameter, resulting from the polysaccharide 55 structure’s elongation, is not taken into consideration for the purposes of determining the apparent peak wet tensile stress of a polysaccharide structure. The apparent peak wet tensile stress of the polysaccharide structures is proportional to their wet tensile strength and is used herein to quantitatively estimate the latter.

“Weight average molecular weight” as used herein means the weight average molecular weight as determined using gel permeation chromatography according to the protocol found in Colloids and Surfaces A: Physico Chemical & Engineering 60 Aspects, Vol. 162, 2000, pg. 107-121.

“Polymer” as used herein means one or more, often repeating molecular units that are covalently bound together via a

C—C bond. Polymers generally include, but are not limited to, homopolymers, copolymers, such as for example, block, graft, random and alternating copolymers, terpolymers, etc., and blends and modifications thereof. In addition, unless otherwise specifically limited, the term "polymer" includes all possible geometric configurations of the material. The configurations include, but are not limited to, isotactic, atactic, syndiotactic, and random symmetries.

"Spinning process temperature" as used herein means the temperature at which the unsubstituted polysaccharide-containing structures in the form of fibers are attenuated at the external surface of the spinning die as the unsubstituted polysaccharide-containing structures are formed.

#### Fibers

The fibers comprising an unsubstituted polysaccharide of the present invention may be continuous or substantially continuous. A fiber is continuous if it extends 100% of the MD length of the web structure and/or web product made therefrom. In one example, a fiber is substantially continuous if it extends greater than about 30% and/or greater than about 50% and/or greater than about 70% of the MD length of the web structure and/or web product made therefrom.

The fibers comprising an unsubstituted polysaccharide of the present invention may be produced by crosslinking polysaccharides together. Nonlimiting examples of a suitable crosslinking system for achieving crosslinking of the polysaccharide comprises a crosslinking agent and optionally a crosslinking facilitator, wherein the polysaccharide is crosslinked by the crosslinking agent. An example of a suitable crosslinking system for use in the present invention is described in U.S. Patent Application Publication 2004/0249066.

In one example, a fiber comprising an unsubstituted polysaccharide of the present invention, as a whole, exhibits no melting point. In other words, it degrades before melting.

In addition to the fibers comprising an unsubstituted polysaccharide of the present invention, other fibers may be included in the webs of the present invention. For example, the webs may include pulp fibers, such as cellulose fibers, fibers comprising substituted polysaccharides, and/or polymer fibers.

In one example of the present invention, a fiber comprising an unsubstituted polysaccharide of the present invention exhibits an apparent peak wet tensile stress greater than 0.2 MPa and/or greater than 0.5 MPa and/or greater than 1 MPa and/or

In another example of the present invention, a fiber comprising an unsubstituted polysaccharide of the present invention comprises at least about 50% and/or at least about 60% and/or at least about 70% to about 100% and/or to about 95% and/or to about 90% by weight of the fiber of an unsubstituted polysaccharide.

In another example of the present invention, a fiber comprising an unsubstituted polysaccharide of the present invention exhibits a pH of less than about 7 and/or less than about 6 and/or less than about 5 and/or less than about 4.5 and/or less than about 4.

In another example of the present invention, a fiber comprising an unsubstituted polysaccharide of the present invention comprises a substitution agent. The substitution agent may be separate and discrete from the unsubstituted polysaccharide. In other words, the substitution agent may not be covalently bound to an oxygen atom of an original hydroxyl moiety of the unsubstituted polysaccharide unless that oxygen atom forms part of a crosslink.

#### Unsubstituted Polysaccharides

Unsubstituted polysaccharides in accordance with the present invention include any unsubstituted polysaccharide that can be incorporated into a polysaccharide structure of the present invention, preferably in the form of a fiber or filament.

Nonlimiting examples of unsubstituted polysaccharides in accordance with the present invention include starch, chitosan, gums, arabinans, and galactans.

The unsubstituted polysaccharides of the present invention may have a weight average molecular weight of greater than about 10,000 g/mol and/or greater than about 40,000 g/mol and/or from about 10,000 to about 80,000,000 g/mol and/or from about 10,000 to about 40,000,000 g/mol and/or from about 10,000 to about 10,000,000 g/mol. Higher and lower molecular weight polysaccharides may be used in combination.

The unsubstituted polysaccharides of the present invention may be subjected to a substitution agent, such as an alkaline agent and/or an acidic agent so long as the hydroxyl moieties of the unsubstituted polysaccharides are not irreversibly derivatized with a substitution agent, unless that hydroxyl moiety is part of a crosslink. For example, an unsubstituted polysaccharide present in a polysaccharide-containing composition comprises an unsubstituted hydroxyl moiety originally that may be substituted with a substitution agent and then converted back to its original unsubstituted state in the polysaccharide structure.

In another example, the unsubstituted polysaccharide of the present invention comprises starch. The starch may be acid thinned starch and/or alkaline cooked starch. The starch may be derived from corn, potato, wheat, tapioca and the like. The weight ratio of amylose to amylopectin in the starch may be from about 10:90 to about 99:1 respectively. In one example, the starch comprises from at least about 10% and/or at least about 20% to about 99% and/or to about 90% by weight of amylose.

A natural starch can be reversibly substituted via chemical and/or enzymatic processes. For example, the natural starch can be acid-thinned, hydroxy-ethylated or hydroxy-propylated or oxidized so long at the hydroxyl moieties are not irreversibly derivatized.

#### Substitution Agents

The unsubstituted polysaccharides of the present invention, particularly the hydroxyl moieties thereof, may be substituted by reacting the unsubstituted polysaccharides with one or more substitution agents so long as the substitutions do not remain in the polysaccharide structures formed from the polysaccharides.

In one example, the substitution agent is a cationic agent. The cationic agent may be selected from the group consisting of: quaternary ammonium compounds, quaternary alkyl amines, quaternary aryl amines, imidizolinium quats, polyethoxylated quaternary alkyl amines and mixture thereof.

Nonlimiting examples of suitable substitution agents include quaternary ammonium compounds, amine oxides and amines.

Nonlimiting examples of quaternary ammonium compounds include dodecyltrimethylammonium chloride, stearyltrimethylammonium chloride, stearyldimethylbenzylammonium chloride, didodecyltrimethylammonium chloride, tetraethylammonium chloride, polyethoxylated quaternary ammonium chloride such as Ethoquad C/12 from Akzo Nobel Chemicals Inc. A suitable quaternary ammonium compound is commercially available from Akzo Nobel Chemicals Inc. under the tradename Arquad 12-50.

Nonlimiting examples of amine oxides include cetyltrimethylamine oxide, lauryldimethylamine oxide, cocamidopropylamine oxide. A suitable amine oxide is commercially available from Stepan Company under the tradename Ammonyl CO.

Nonlimiting examples of amines, such as alkyl amines, include ethoxylated dodecylamine, ethoxylated stearylamine, and ethoxylated oleylamine. A suitable amine is commercially available from Akzo Nobel Chemicals Inc. under the tradename Ethomeen C/12.

#### Polysaccharide-Containing Composition

The polysaccharide-containing composition of the present invention may comprise an unsubstituted polysaccharide. The polysaccharide-containing composition may be a mixture of polysaccharides and optionally polymers, wherein at least one is an unsubstituted polysaccharide, and/or fillers both inorganic and organic, and/or fibers and/or foaming agents.

The polysaccharide-containing composition may already be formed. In one example, an unsubstituted polysaccharide may be solubilized via contact with a liquid, such as water, in order to form an unsubstituted polysaccharide-containing composition. Such a liquid may be considered for the purposes of the present invention as performing the function of an external plasticizer. Alternatively, any other suitable processes known to those skilled in the art to produce the polysaccharide-containing composition such that the polysaccharide-containing composition exhibits suitable properties for processing the composition into an polysaccharide structure in accordance with the present invention may be used.

The polysaccharide-containing composition may have and/or be exposed to a temperature of from about 23° C. to about 100° C. and/or from about 65° C. to about 95° C. and/or from about 70° C. to about 90° C. when making polysaccharide structures from the polysaccharide-containing composition. The polysaccharide-containing composition may have and/or be exposed to a temperature that is generally higher when making film and/or foam polysaccharide structures, as described below.

The pH of the polysaccharide-containing composition may be from about 2.5 to about 10 and/or from about 3 to about 9.5 and/or from about 3 to about 8.5 and/or from about 3.2 to about 8 and/or from about 3.2 to about 7.5.

In another example, a polysaccharide-containing composition of the present invention may comprise at least about 5% and/or at least about 15% and/or from at least about 20% and/or 30% and/or 40% and/or 45% and/or 50% to about 75% and/or 80% and/or 85% and/or 90% and/or 95% and/or 99.5% by weight of the polysaccharide-containing composition of a substituted or unsubstituted polysaccharide.

The polysaccharide may have a weight average molecular weight greater than about 10,000 g/mol prior to crosslinking.

A crosslinking system may be present in the polysaccharide-containing composition and/or may be added to the polysaccharide-containing composition before processing the polysaccharide-containing composition into an polysaccharide structure.

The polysaccharide-containing composition may comprise a) at least about 5% and/or at least about 15% and/or from at least about 20% and/or 30% and/or 40% and/or 45% and/or 50% to about 75% and/or 80% and/or 85% by weight of the polysaccharide-containing composition of a polysaccharide; b) a crosslinking system comprising from about 0.1% to about 10% by weight of the polysaccharide-containing composition of a crosslinking agent; and c) from about

10% and/or 15% and/or 20% to about 50% and/or 55% and/or 60% and/or 70% by weight of the polysaccharide-containing composition of external plasticizer e.g., water.

The crosslinking system of the present invention may further comprise, in addition to the crosslinking agent, a crosslinking facilitator.

“Crosslinking facilitator” as used herein means any material that is capable of activating a crosslinking agent thereby transforming the crosslinking agent from its unactivated state to its activated state.

Upon crosslinking the polysaccharide, the crosslinking agent becomes an integral part of the polysaccharide structure as a result of crosslinking the polysaccharide as shown in the following schematic representation:

15 Polysaccharide—Crosslinking agent—Polysaccharide

The crosslinking facilitator may include derivatives of the material that may exist after the transformation/activation of the crosslinking agent. For example, a crosslinking facilitator salt being chemically changed to its acid form and vice versa.

20 Nonlimiting examples of suitable crosslinking facilitators include acids having a pKa of between 2 and 6 or salts thereof. The crosslinking facilitators may be Bronsted Acids and/or salts thereof, for example ammonium salts thereof.

In addition, metal salts, such as magnesium and zinc salts, can be used alone or in combination with Bronsted Acids and/or salts thereof, as crosslinking facilitators.

25 Nonlimiting examples of suitable crosslinking facilitators include acetic acid, benzoic acid, citric acid, formic acid, glycolic acid, lactic acid, maleic acid, phthalic acid, phosphoric acid, succinic acid and mixtures thereof and/or their salts, preferably their ammonium salts, such as ammonium glycolate, ammonium citrate, ammonium sulfate, and ammonium chloride.

#### 30 Polymers

Polymers may be used in combination with the polysaccharides of the present invention to form the polysaccharide structures of the present invention. The polymers may be unsubstituted or substituted.

35 Polyvinylalcohols, which are suitable for use in combination with one or more polysaccharides of the present invention, are characterized by the following general formula:

45

Structure I



50 each R is selected from the group consisting of C<sub>1</sub>-C<sub>4</sub> alkyl; C<sub>1</sub>-C<sub>4</sub> acyl; and x/x+y+z=0.5-1.0. In one example, the polyvinylalcohol has no “y” and/or “z” units.

55 Polyvinyl alcohols herein can be grafted with other monomers to modify its properties. A wide range of monomers has been successfully grafted to polyvinyl alcohol. Nonlimiting examples of such monomers include vinyl acetate, styrene, acrylamide, acrylic acid, 2-hydroxyethyl methacrylate, acrylonitrile, 1,3-butadiene, methyl methacrylate, methacrylic acid, vinylidene chloride, vinyl chloride, vinyl amine and a variety of acrylate esters.

60 “Petroleum-derived polymers” as used herein means any polymer that has been obtained from petroleum. Nonlimiting examples of such petroleum-derived polymers include polyolefins. Nonlimiting examples of polyolefins include polypropylene, polyethylene, polyesters, and the like.

“Polyvinylamines” as used herein means any hydrocarbon polymer that comprises amino groups.

#### Synthesis of Polysaccharide-Containing Composition

A polysaccharide-containing composition of the present invention may be prepared using a screw extruder, such as a vented twin screw extruder.

A barrel **10** of an APV Baker (Peterborough, England) twin screw extruder is schematically illustrated in FIG. 1A. The barrel **10** is separated into eight zones, identified as zones **1-8**. The barrel **10** encloses the extrusion screw and mixing elements, schematically shown in FIG. 1B, and serves as a containment vessel during the extrusion process. A solid feed port **12** is disposed in zone **1** and a liquid feed port **14** is disposed in zone **1**. A vent **16** is included in zone **7** for cooling and decreasing the liquid, such as water, content of the mixture prior to exiting the extruder. An optional vent stuffer, commercially available from APV Baker, can be employed to prevent the polysaccharide-containing composition from exiting through the vent **16**. The flow of the polysaccharide-containing composition through the barrel **10** is from zone **1** exiting the barrel **10** at zone **8**.

A screw and mixing element configuration for the twin screw extruder is schematically illustrated in FIG. 1B. The

threaded in the opposite direction, are used in order to control flow and corresponding mixing time.

In zone **1**, an unsubstituted polysaccharide is fed into the solid feed port at a rate of 230 grams/minute using a K-Tron (Pitman, N.J.) loss-in-weight feeder. This unsubstituted polysaccharide is combined inside the extruder (zone **1**) with water, an external plasticizer, added at the liquid feed at a rate of 146 grams/minute using a Milton Roy (Ivyland, Pa.) diaphragm pump (1.9 gallon per hour pump head) to form an unsubstituted polysaccharide/water slurry. This slurry is then conveyed down the barrel of the extruder and cooked, in the presence of an alkaline agent, such as ammonium hydroxide and/or sodium hydroxide. The cooking causes a hydrogen from at least one hydroxyl moiety on the unsubstituted polysaccharide to become disassociated with the hydroxyl moiety and thus create a negative charge on the oxygen atom of the former hydroxyl moiety. This oxygen atom is now open for substitution by a substitution agent, such as a quaternary ammonium compound, for example a quaternary amine. Accordingly, a substitution agent is added to the unsubstituted polysaccharide mixture, thus creating a substituted polysaccharide.

Table 1 describes the temperature, pressure, and corresponding function of each zone of the extruder.

TABLE I

| Zone | Temp.(° F.) | Pressure | Description of Screw         | Purpose                              |
|------|-------------|----------|------------------------------|--------------------------------------|
| 1    | 70          | Low      | Feeding/Conveying            | Feeding and Mixing                   |
| 2    | 70          | Low      | Conveying                    | Mixing and Conveying                 |
| 3    | 70          | Low      | Conveying                    | Mixing and Conveying                 |
| 4    | 130         | Low      | Pressure/Decreased Conveying | Conveying and Heating                |
| 5    | 300         | Medium   | Pressure Generating          | Cooking at Pressure and Temperature  |
| 6    | 250         | High     | Reversing                    | Cooking at Pressure and Temperature  |
| 7    | 210         | Low      | Conveying                    | Cooling and Conveying (with venting) |
| 8    | 210         | Low      | Pressure Generating          | Conveying                            |

twin screw extruder comprises a plurality of twin lead screws (TLS) (designated A and B) and single lead screws (SLS) (designated C and D) installed in series. Screw elements (A-D) are characterized by the number of continuous leads and the pitch of these leads.

A lead is a flight (at a given helix angle) that wraps the core of the screw element. The number of leads indicates the number of flights wrapping the core at any given location along the length of the screw. Increasing the number of leads reduces the volumetric capacity of the screw and increases the pressure generating capability of the screw.

The pitch of the screw is the distance needed for a flight to complete one revolution of the core. It is expressed as the number of screw element diameters per one complete revolution of a flight. Decreasing the pitch of the screw increases the pressure generated by the screw and decreases the volumetric capacity of the screw.

The length of a screw element is reported as the ratio of length of the element divided by the diameter of the element.

This example uses TLS and SLS. Screw element A is a TLS with a 1.0 pitch and a 1.5 length ratio. Screw element B is a TLS with a 1.0 pitch and a 1.0 L/D ratio. Screw element C is a SLS with a 1/4 pitch and a 1.0 length ratio. Screw element D is a SLS and a 1/4 pitch and a 1/2 length ratio.

Bilobal paddles, E, serving as mixing elements, are also included in series with the SLS and TLS screw elements in order to enhance mixing. Various configurations of bilobal paddles and reversing elements F, single and twin lead screws

40 After the slurry exits the extruder, part of the substituted polysaccharide/water slurry can be dumped and another part (100 g) can be fed into a Zenith®, type PEP II (Sanford N.C.) and pumped into a SMX style static mixer (Koch-Glitsch, Woodridge, Ill.). The static mixer is used to combine additional additives such as polymers, crosslinking agents, 45 crosslinking facilitators, external plasticizers, such as water, with the substituted polysaccharide/water slurry to form a substituted polysaccharide-containing composition. The additives are pumped into the static mixer via PREP 100 HPLC pumps (Chrom Tech, Apple Valley, Minn.). These pumps provide high pressure, low volume addition capability. The substituted polysaccharide-containing composition of the present invention is ready to be processed into an polysaccharide structure.

50 55 Processing

“Processing” as used herein means any operation and/or process by which an polysaccharide structure comprising an unsubstituted polysaccharide is formed from a polysaccharide-containing composition.

60 Nonlimiting examples of processing operations include extrusion, molding and/or fiber spinning. Extrusion and molding (either casting or blown), typically produce films, sheets and various profile extrusions. Molding may include injection molding, blown molding and/or compression molding. Fiber spinning may include spun bonding, melt blowing, continuous filament producing and/or tow fiber producing.

## Polysaccharide Structure

The polysaccharide-containing composition can be subjected to one or more processing operations such that the polysaccharide-containing composition is processed into an polysaccharide structure comprising an unsubstituted polysaccharide and optionally, a crosslinking system, according to the present invention.

The crosslinking system via the crosslinking agent crosslinks polysaccharides together to produce the polysaccharide structure of the present invention, with or without being subjected to a curing step. In other words, the crosslinking system in accordance with the present invention acceptably crosslinks the polysaccharides together via the crosslinking agent to form a unitary polysaccharide structure. The crosslinking agent is a "building block" for the polysaccharide structure. Without the crosslinking agent, no polysaccharide structure in accordance with the present invention could be formed.

Polysaccharide structures of the present invention do not include coatings and/or other surface treatments that are applied to a pre-existing form, such as a coating on a fiber, film or foam.

In one example, the polysaccharide structure produced via a processing operation may be cured at a curing temperature of from about 110° C. to about 200° C. and/or from about 120° C. to about 195° C. and/or from about 130° C. to about 185° C. for a time period of from about 0.01 and/or 1 and/or 5 and/or 15 seconds to about 60 minutes and/or from about 20 seconds to about 45 minutes and/or from about 30 seconds to about 30 minutes. Alternative curing methods may include radiation methods such as UV, e-beam, IR and other temperature-raising methods.

Further, the polysaccharide structure may also be cured at room temperature for days, either after curing at above room temperature or instead of curing at above room temperature.

The polysaccharide structure may exhibit an initial total wet tensile, as measured by the Initial Total Wet Tensile Test Method described herein, of at least about 1.18 g/cm (3 g/in) and/or at least about 1.97 g/cm (5 g/in) and/or at least about 5.91 g/cm (15 g/in) and/or at least about 9.84 g/cm (25 g/in) to about 51.18 g/cm (130 g/in) and/or to about 43.31 g/cm (110 g/in) and/or to about 35.43 g/cm (90 g/in) and/or to about 25.53 g/cm (75 g/in) and/or to about 23.62 g/cm (60 g/in) and/or to about 21.65 g/cm (55 g/in) and/or to about 19.69 g/cm (50 g/in).

In one example, an polysaccharide structure of the present invention may comprise from at least about 20% and/or 30% and/or 40% and/or 45% and/or 50% to about 75% and/or 80% and/or 85% and/or 90% and/or 95% and/or 99.5% by weight of the polysaccharide structure of a polysaccharide.

## Synthesis of an Polysaccharide Structure

Nonlimiting examples of processes for preparing polysaccharide structures comprising an unsubstituted polysaccharide in accordance with the present invention follow.

## i) Fiber Formation

A polysaccharide-containing composition is prepared according to the Synthesis of a Polysaccharide-Containing Composition described above. As shown in FIG. 2, the polysaccharide-containing composition may be processed into a polysaccharide structure comprising an unsubstituted polysaccharide. The polysaccharide-containing composition present in an extruder 102 is pumped to a die 104 using pump 103, such as a Zenith®, type PEP II, having a capacity of 0.6 cubic centimeters per revolution (cc/rev), manufactured by Parker Hannifin Corporation, Zenith Pumps division, of Sanford, N.C., USA. The flow of the polysaccharide, such as

starch, to die 104 is controlled by adjusting the number of revolutions per minute (rpm) of the pump 103. Pipes connecting the extruder 102, the pump 103, the die 104, and optionally a mixer 116 are electrically heated and thermostatically controlled to 65° C.

The die 104 has several rows of circular extrusion nozzles 200 spaced from one another at a pitch P (FIG. 3) of about 1.524 millimeters (about 0.060 inches). The nozzles 200 have individual inner diameters D2 of about 0.305 millimeters (about 0.012 inches) and individual outside diameters (D1) of about 0.813 millimeters (about 0.032 inches). Each individual nozzle 200 is encircled by an annular and divergently flared orifice 250 formed in a plate 260 (FIGS. 3 and 4) having a thickness of about 1.9 millimeters (about 0.075 inches). A pattern of a plurality of the divergently flared orifices 250 in the plate 260 correspond to a pattern of extrusion nozzles 200. The orifices 250 have a larger diameter D4 (FIGS. 3 and 4) of about 1.372 millimeters (about 0.054 inches) and a smaller diameter D3 of 1.17 millimeters (about 0.046 inches) for 10 attenuation air. The plate 260 was fixed so that the embryonic fibers 110 being extruded through the nozzles 200 are surrounded and attenuated by generally cylindrical, humidified air streams supplied through the orifices 250. The nozzles can extend to a distance from about 1.5 mm to about 4 mm, and more specifically from about 2 mm to about 3 mm, beyond a surface 261 of the plate 260 (FIG. 3). As shown in FIG. 5, a plurality of boundary-air orifices 300, is formed by plugging nozzles of two outside rows on each side of the plurality of nozzles, as viewed in plane, so that each of the boundary-layer orifice comprised a annular aperture 250 described herein above. Additionally, every other row and every other column of the remaining capillary nozzles are blocked, increasing the spacing between active capillary nozzles

As shown in FIG. 2, attenuation air can be provided by 35 heating compressed air from a source 106 by an electrical-resistance heater 108, for example, a heater manufactured by Chromalox, Division of Emerson Electric, of Pittsburgh, Pa., USA. An appropriate quantity of steam 105 at an absolute pressure of from about 240 to about 420 kiloPascals (kPa), 40 controlled by a globe valve (not shown), is added to saturate or nearly saturate the heated air at the conditions in the electrically heated, thermostatically controlled delivery pipe 115. Condensate is removed in an electrically heated, thermostatically controlled, separator 107. The attenuating air has an 45 absolute pressure from about 130 kPa to about 310 kPa, measured in the pipe 115. The fibers 110 being extruded have a moisture content of from about 20% and/or 25% to about 50% and/or 55% by weight. The fibers 110 are dried by a 50 drying air stream 109 having a temperature from about 149° C. (about 300° F.) to about 315° C. (about 600° F.) by an electrical resistance heater (not shown) supplied through drying nozzles 112 and discharged at an angle generally perpendicular relative to the general orientation of the embryonic fibers being extruded. The fibers are dried from about 55 45% moisture content to about 15% moisture content (i.e., from a consistency of about 55% to a consistency of about 85%) and are collected on a collection device 111, such as, for example, a movable foraminous belt.

The process parameters are as follows.

60

| Sample                      | Units |
|-----------------------------|-------|
| Attenuation Air Flow Rate   | G/min |
| Attenuation Air Temperature | °C.   |
| Attenuation Steam Flow Rate | G/min |

65

2500

93

500

-continued

| Sample                                     | Units      |           |
|--------------------------------------------|------------|-----------|
| Attenuation Steam Gage Pressure            | kPa        | 213       |
| Attenuation Gage Pressure in Delivery Pipe | kPa        | 26        |
| Attenuation Exit Temperature               | ° C.       | 71        |
| Solution Pump Speed                        | Revs/min   | 35        |
| Solution Flow                              | G/min/hole | 0.18      |
| Drying Air Flow Rate                       | g/min      | 10200     |
| Air Duct Type                              |            | Slots     |
| Air Duct Dimensions                        | Mm         | 356 x 127 |
| Velocity via Pitot-Static Tube             | M/s        | 34        |
| Drying Air Temperature at Heater           | ° C.       | 260       |
| Dry Duct Position from Die                 | Mm         | 80        |
| Drying Duct Angle Relative to Fibers       | degrees    | 0         |

### ii) Foam Formation

The polysaccharide-containing composition for foam formation is prepared similarly as for fiber formation except that the water content will be less, typically from about 10-21% of the substituted or unsubstituted polysaccharide weight. With less water to plasticize the polysaccharide, higher temperatures may be needed in extruder zones 5-8 (FIG. 1A), typically from 150-250° C. Also with less water available, it may be necessary to add the crosslinking system, especially the crosslinking agent, with the water in zone 1. In order to avoid premature crosslinking in the extruder, the polysaccharide-containing composition pH should be between 7 and 8, achievable by using a crosslinking facilitator e.g., ammonium salt. A die is placed at the location where the extruded material emerges and is typically held at 160-210° C. Modified high amylose starches (for example greater than 50% and/or greater than 75% and/or greater than 90% by weight of the starch of amylose) granulated to particle sizes ranging from 400-1500 microns are preferred for this application. It may also be advantageous to add a nucleating agent such as micro-talc or alkali metal or alkaline earth metal salt such as sodium sulfate or sodium chloride in an amount of about 1-8% of the starch weight. The foam may be shaped into various forms.

### iii) Film Formation

The polysaccharide-containing composition for film formation is prepared similarly as for foam formation except that the added water content is less, typically 3-15% of the substituted or unsubstituted polysaccharide weight and a polyol external plasticizer such as glycerol is included at 10-30% of the polysaccharide weight. As with foam formation, zones 5-7 (FIG. 1A) are held at 160-210° C., however, the slit die temperature is lower between 60-120° C. As with foam formation, the crosslinking system, especially the crosslinking agent, may be added along with the water in zone 1 and the polysaccharide-containing composition pH should be between 7-8 achievable by using a crosslinking facilitator e.g., ammonium salt.

Films of the present invention may be utilized for any suitable products known in the art. For example, the films may be used in packaging materials.

### Process for Making Polysaccharide Structures

The polysaccharide structures of the present invention may be made by any suitable process known to those skilled in the art.

A nonlimiting example of a suitable process for making an unsubstituted polysaccharide structure according to the present invention comprises the step of obtaining an polysaccharide structure comprising an unsubstituted polysaccharide

from a polysaccharide-containing composition comprising a substituted form of the unsubstituted polysaccharide.

In still another example of the present invention, a process for making an polysaccharide structure comprising an unsubstituted polysaccharide, wherein the process comprises the step of processing a polysaccharide-containing composition comprising an unsubstituted polysaccharide into an polysaccharide structure comprising the unsubstituted polysaccharide, is provided.

10 In even yet another example of the present invention, a process for making an polysaccharide structure comprising an unsubstituted polysaccharide, wherein the process comprises the steps of:

15 a. providing a polysaccharide-containing composition comprising an unsubstituted polysaccharide;

b. substituting the unsubstituted polysaccharide to produce a substituted polysaccharide; and

20 c. processing the polysaccharide-containing composition comprising the substituted polysaccharide into an polysaccharide structure comprising the unsubstituted polysaccharide, is provided.

25 In one example, an unsubstituted polysaccharide, specifically one or more hydroxyl moieties present on the unsubstituted polysaccharide, is substituted with a moiety for a time sufficient to permit an polysaccharide structure comprising the unsubstituted polysaccharide to be formed from the substituted polysaccharide. In other words, without wishing to be bound by theory, the substitution agent temporarily impacts the properties of the unsubstituted polysaccharide in a manner such that it can be spun and/or otherwise processed into an polysaccharide structure, such as a fiber. Before, during and/or after the polysaccharide structure is formed, the substitution agent is replaced by a hydroxyl moiety, thus returning the polysaccharide to an unsubstituted form wherein the previously substituted oxygen of the hydroxyl moiety is now covalently bonded to a hydrogen.

30 The substituting step may comprise subjecting the unsubstituted polysaccharide to an alkaline pH. For example, the substituting step may comprise subjecting the unsubstituted polysaccharide to a pH of greater than 7 and/or at least about 7.5 and/or at least about 8 and/or at least about 8.5. To achieve the alkaline pH, an alkaline agent may be used in the substituting step. Nonlimiting examples of suitable alkaline agents may be selected from the group consisting of sodium hydroxide, calcium hydroxide, magnesium hydroxide, potassium hydroxide, ammonium hydroxide and mixtures thereof. Further, the substituting step may occur at a temperature in the range of from about 70° C. to about 120° C. and/or from about 75° C. to about 100° C.

35 40 45 50 The substituting step may comprise reacting the unsubstituted polysaccharide with a substitution agent to form a substituted polysaccharide.

55 The step of obtaining a fiber from the substituted polysaccharide may comprise subjecting the substituted polysaccharide to an acidic pH. For example, the step of obtaining a fiber from the substituted polysaccharide may comprise subjecting the substituted polysaccharide to a pH of less than 7 and/or less than about 6 and/or less than about 5 and/or less than about 4.5 and/or less than about 4. To achieve the acidic pH, an acidic agent may be used in the obtaining a fiber step. Nonlimiting examples of suitable acidic agents may be selected from the group consisting of: acetic acid, benzoic acid, citric acid, formic acid, glycolic acid, lactic acid, maleic acid, phthalic acid, phosphoric acid, succinic acid and mixtures thereof and/or their salts, preferably their ammonium salts, such as ammonium glycolate, ammonium citrate, ammonium sulfate, ammonium chloride, and mixtures

thereof. Further, the obtaining a fiber step may occur at a temperature in the range of from about 60° C. to about 100° and/or from about 70° C. to about 95° C.

The step of obtaining a polysaccharide structure may comprise spinning the substituted polysaccharide such that a fiber comprising an unsubstituted polysaccharide is formed. The spinning may be any suitable spinning operation known to those skilled in the art.

The process of the present invention may further comprise a step of collecting a plurality of the fibers to form a web.

#### Test Methods

All tests described herein including those described under the Definitions section and the following test methods are conducted on samples that have been conditioned in a conditioned room at a temperature of 73° F.±4° F. (about 23° C.±2.2° C.) and a relative humidity of 50%±10% for 24 hours prior to the test. Further, all tests are conducted in such conditioned room. Tested samples and felts should be subjected to 73° F.±4° F. (about 23° C.±2.2° C.) and a relative humidity of 50%±10% for 24 hours prior to capturing images.

#### A. Apparent Peak Wet Tensile Stress Test Method

The following test has been designed to measure the apparent peak wet tensile stress of a starch fiber during the first minutes of the fiber being moistened—to reflect a consumer's real-life expectations as to the strength properties of the end product, such as, for example, a toilet tissue, during its use.

##### (A) Equipment:

Sunbeam® ultrasonic humidifier, Model 696-12, manufactured by Sunbeam Household Products Co. of McMinnville, Tenn., USA. The humidifier has an on/off switch and is operated at room temperature. A 27-inch length of 0.625" OD 0.25" ID rubber hose was attached to an output. When operating correctly, the humidifier will output between 0.54 and 0.66 grams of water per minute as a mist.

The water droplet velocity and the water droplet diameter of the mist generated by the humidifier can be measured using photogrammetric techniques. Images can be captured using a Nikon®, Model D1, of Japan, 3-megapixel digital camera equipped with a 37 mm coupling ring, a Nikon® PB-6 bellows, and a Nikon® auto-focus AF Micro Nikkor® 200 mm 1:4 D lens. Each pixel had the dimension of about 3.5 micrometer assuming a square pixel. Images can be taken in shadow mode using a Nano Twin Flash (High-Speed Photo-Systeme, of Wedel, Germany). Any number of commercially available image-processing packages can be used to process the images. The dwell time between the two flashes of this system is set at 5, 10, and 20 microsecond. The distance traveled by water droplets between flashes is used to calculate droplet velocity.

Water droplets were found to be from about 12 microns to about 25 microns in diameter. The velocity of the water droplets at a distance of about (25±5) mm from the outlet of the flexible hose was calculated to be about 27 meters per second (m/sec), ranging from about 15 m/sec to about 50 m/sec. Obviously, as the mist stream encountered room air, the velocity of the water droplets slows with increasing distance from the hose exit due to drag forces.

The flexible hose is positioned so that the mist stream totally engulfs the fiber thereby thoroughly wetting the fiber. To ensure that the fiber is not damaged or broken by the mist stream, the distance between the outlet of the flexible hose and the fiber is adjusted until the mist stream stalls at or just past the fiber.

Filament Stretching Rheometer (FSR) with 1-gram Force Transducer, Model 405A, manufactured by Aurora Scientific Inc., of Aurora, Ontario, Canada, equipped with small metal hook. Initial instrument settings are:

---

|                         |                                   |
|-------------------------|-----------------------------------|
| initial gap = 0.1 cm    | strain rate = 0.1 s <sup>-1</sup> |
| Hencky strain limit = 4 | data points per second = 25       |
| post move time = 0      |                                   |

---

10

FSR is based on a design similar to that described in an article titled "A Filament Stretching Device For Measurement Of Extensional Viscosity," published by J. Rheology 37 (6), 1993, pages 1081-1102 (Tirtaatmadja and Sridhar), incorporated herein by reference, with the following modifications:

- (a) FSR is oriented so that the two end plates can move in a vertical direction.
- (b) FSR comprises two independent ball screw linear actuators, Model PAG001 (manufactured by Industrial Device Corp. of Petaluma, Calif., USA), each actuator driven by a stepper motor (for example, Zeta® 83-135, manufactured by Parker Hannifin Corp., Compumotor Division, Rohnert Park, Calif., USA). One of the motors can be equipped with an encoder (for example, Model E151000C865, manufactured by Dynapar Brand, Danaher Controls of Gurnee, Ill., USA) to track the position of the actuator. The two actuators can be programmed to move equal distances at equal speeds in opposite directions.

- (c) The maximal distance between the end plates is approximately 813 mm (about 32 inches).

A wide-bandwidth single-channel signal-conditioning module, Model 5B41-06, manufactured by Analog Devices Co. of Norwood, Mass., USA can be used to condition the signal from the force transducer, Model 405A, manufactured by Aurora Scientific Inc., of Aurora, Ontario, Canada.

#### Example of Fibers Comprising an Unsubstituted Polysaccharide and Method for Determining Apparent Peak Wet Tensile Stress Thereof

Twenty five grams of an unsubstituted polysaccharide, for example Eclipse G starch (acid thinned dent corn starch of approximate average molecular weight of 3,000,000 g/mol, from A. E. Staley Manufacturing Corporation of Decatur, Ill., USA), 10.00 grams of a polysaccharide, for example 10% Celvol 310 solution in water (Ethenol, homopolymer from Celanese Ltd. Dallas Tex., USA) (4% based on the weight of the starch), 1.00 grams of an alkaline agent, for example 25% Sodium hydroxide solution (1% based on the weight of starch), 0.67 g of a substitution agent, for example Arquad 12-37W (Trimethylodecylammonium chloride from Akzo Nobel Chemicals Inc. of Chicago, Ill., USA) (1% based on the weight of the starch), and 50 grams of water are added to a 200 ml beaker. The beaker is disposed in a water bath to boil for approximately one hour while the starch mix is stirred manually to destructure the starch and to evaporate the amount of water until about 25 grams of water remain in the breaker.

Then 1.66 grams of a crosslinking agent, for example Parez® 490 from Lanxess Corp. (formerly Bayer Corp.), Pittsburgh, Pa., USA, (3% urea-glyoxal resin based on the weight of the starch), and 4.00 grams of a crosslinking facilitator, for example 25% Ammonium chloride solution (4% based on the weight of the starch) are added to the beaker and mixed. Then the mixture is cooled to a temperature of about 40° C. A portion of the mixture is transferred to a 10 cubic centimeter (cc) syringe and is extruded therefrom to form a

45

50

55

60

65

fiber. The fiber is manually elongated so that the fiber has a diameter between about 10  $\mu\text{m}$  and about 100  $\mu\text{m}$ . Then, the fiber is suspended in an ambient air for approximately one minute to allow the fiber to dry and solidify. The fiber is placed on an aluminum pan and is cured in a convection oven for about 10 minutes at a temperature of about 130° C. The cured fiber is then placed in a room having a constant temperature of about 22° C. and a constant relative humidity of about 25% for about 24 hours.

Since the single fibers are fragile, a coupon 90 (FIG. 6) can be used to support the fiber 110. The coupon 90 can be manufactured from an ordinary office copy paper or a similar light material. In an illustrative example of FIG. 6, the coupon 90 comprises a rectangular structure having the overall size of about 20 millimeters by about 8 millimeters, with a rectangle cutout 91 sized about 9 millimeters by about 5 millimeters in the center of the coupon 90. The ends 110a, 110b of the fiber 110 can be secured to the ends of the coupon 90 with an adhesive tape 95 (such as, for example, a conventional Scotch tape), or otherwise, so that the fiber 110 spans the distance (of about 9 millimeters in the instant example) of the cut-out 91 in the center of the coupon 90, as shown in FIG. 6. For convenience of mounting, the coupon 90 may have a hole 98 in the top portion of the coupon 90, structured to receive a suitable hook mounted on the upper plate of the force transducer. Prior to applying a force to the fiber, the fiber's diameter can be measured with an optical microscope at 3 positions and averaged to obtain the average fiber diameter used in calculations.

The coupon 90 can then be mounted onto a fiber-stretching rheometer (not shown) so that the fiber 110 is substantially parallel to the direction of the load "P" (FIG. 6) to be applied. Side portions of the coupon 90 that are parallel to the fiber 110 can be cut (along lines 92, FIG. 6), so that the fiber 110 is the only element receiving the load. Then the fiber 110 can be sufficiently moistened. For example, an ultrasonic humidifier (not shown) can be turned on, with a rubber hose positioned about 200 millimeters (about 8 inches) away from the fiber so as to direct the output mist directly at the fiber. The fiber 110 can be exposed to the vapor for about one minute, after which the force load P can be applied to the fiber 110. The fiber 110 continues to be exposed to the vapor during the application of the force load that imparts elongation force to the fiber 110. Care should be taken to ensure that the fiber 110 is continuously within the main stream of the humidifier output as the force is applied to the fiber. When correctly exposed, droplets of water are typically visible on or around the fiber 110. The humidifier, its contents, and the fiber 110 are allowed to equilibrate to an ambient temperature before use.

Using the force load and diameter measurements, the wet tensile stress can be calculated in units of MegaPascals (MPa). The test can be repeated multiple times, for example eight times. The results of wet tensile stress measurements of eight fibers are averaged. The force readings from the force transducer are corrected for the mass of the residual coupon by subtracting the average force transducer signal collected after the fiber had broken from the entire set of force readings. The stress at failure for the fiber can be calculated by taking the maximum force generated on the fiber divided by the cross-sectional area of the fiber based on the optical microscope measurements of the fiber's average fiber diameter measured prior to conducting the test. The actual beginning plate separation (bps) can be dependent on a particular sample tested, but is recorded in order to calculate the actual engineering strain of the sample. In the instant example, the resulting average wet tensile stress of 0.33 MPa, with the standard deviation of 0.29, was obtained.

#### B. Average Fiber Diameter Test Method

A web comprising fibers of appropriate basis weight (approximately 5 to 20 grams/square meter) is cut into a rectangular shape, approximately 20 mm by 35 mm. The sample is 5 then coated using a SEM sputter coater (EMS Inc, Pa., USA) with gold so as to make the fibers relatively opaque. Typical coating thickness is between 50 and 250 nm. The sample is then mounted between two standard microscope slides and compressed together using small binder clips. The sample is 10 imaged using a 10x objective on an Olympus BHS microscope with the microscope light-collimating lens moved as far from the objective lens as possible. Images are captured using a Nikon D1 digital camera. A Glass microscope micrometer is used to calibrate the spatial distances of the 15 images. The approximate resolution of the images is 1  $\mu\text{m}/\text{pixel}$ . Images will typically show a distinct bimodal distribution in the intensity histogram corresponding to the fibers and the background. Camera adjustments or different basis weights are used to achieve an acceptable bimodal distribution. Typically 10 images per sample are taken and the 20 image analysis results averaged.

The images are analyzed in a similar manner to that described by B. Pourdeyhimi, R. and R. Dent in "Measuring fiber diameter distribution in nonwovens" (Textile Res. J. 25 69(4) 233-236, 1999). Digital images are analyzed by computer using the MATLAB (Version 6.3) and the MATLAB Image Processing Tool Box (Version 3.) The image is first converted into a grayscale. The image is then binarized into 20 black and white pixels using a threshold value that minimizes 30 the intraclass variance of the thresholded black and white pixels. Once the image has been binarized, the image is skeletonized to locate the center of each fiber in the image. The distance transform of the binarized image is also computed. The scalar product of the skeltonized image and the distance 35 map provides an image whose pixel intensity is either zero or the radius of the fiber at that location. Pixels within one radius of the junction between two overlapping fibers are not counted if the distance they represent is smaller than the radius of the junction. The remaining pixels are then used to 40 compute a length-weighted histogram of fiber diameters contained in the image.

#### C. Initial Total Wet Tensile Test Method

An electronic tensile tester (Thwing-Albert EJA Materials Tester, Thwing-Albert Instrument Co., 10960 Dutton Rd., Philadelphia, Pa., 19154) is used and operated at a crosshead speed of 4.0 inch (about 10.16 cm) per minute and a gauge length of 1.0 inch (about 2.54 cm), using a strip of a polysaccharide structure of 1 inch wide and a length greater than 3 inches long. The two ends of the strip are placed in the upper jaws of the machine, and the center of the strip is placed 45 around a stainless steel peg (0.5 cm in diameter). After verifying that the strip is bent evenly around the steel peg, the strip is soaked in distilled water at about 20° C. for a soak time of 55 5 seconds before initiating cross-head movement. The initial result of the test is an array of data in the form load (grams force) versus crosshead displacement (centimeters from starting point).

The sample is tested in two orientations, referred to here as 60 MD (machine direction, i.e., in the same direction as the continuously wound reel and forming fabric) and CD (cross-machine direction, i.e., 90° from MD). The MD and CD wet tensile strengths are determined using the above equipment and calculations in the following manner:

$$\begin{aligned} \text{Initial Total Wet Tensile} &= \text{ITWT(g/inch)} = \text{Peak} \\ &\text{Load}_{\text{MD}}(\text{g})/2(\text{inch}_{\text{width}}) + \text{Peak Load}_{\text{CD}}(\text{g})/2 \\ &(\text{inch}_{\text{width}}) \end{aligned}$$

**19**

The Initial Total Wet Tensile value is then normalized for the basis weight of the strip from which it was tested. The normalized basis weight used is 36 g/m<sup>2</sup>, and is calculated as follows:

$$\text{Normalized}\{\text{ITWT}\} = \{\text{ITWT}\} * 36(\text{g/m}^2) / \text{Basis Weight of Strip(g/m}^2)$$

If the initial total wet tensile of a polysaccharide structure comprising a crosslinking system of the present invention is at least 1.18 g/cm (3 g/in) and/or at least 1.57 g/cm (4 g/in) and/or at least 1.97 g/cm (5 g/in), then the crosslinking system is acceptable and is within the scope of the present invention. Preferably, the initial total wet tensile is less than or equal to about 23.62 g/cm (60 g/in) and/or less than or equal to about 21.65 g/cm (55 g/in) and/or less than or equal to about 19.69 g/cm (50 g/in).

All documents cited in the Detailed Description of the Invention are, in relevant part, incorporated herein by reference; the citation of any document is not to be construed as an admission that it is prior art with respect to the present invention. Terms or phrases defined herein are controlling even if such terms or phrases are defined differently in the incorporated herein by reference documents.

While particular embodiments of the present invention have been illustrated and described, it would be obvious to those skilled in the art that various other changes and modifications can be made without departing from the spirit and scope of the invention. It is therefore intended to cover in the appended claims all such changes and modifications that are within the scope of this invention.

What is claimed is:

**1. A fiber, wherein the fiber comprises an unsubstituted polysaccharide and an amine oxide, wherein the fiber exhibits an apparent peak wet tensile stress greater than 0.2 MPa.**

**20**

**2. The fiber according to claim 1 wherein the unsubstituted polysaccharide has a weight average molecular weight of at least 10,000 g/mol.**

**3. The fiber according to claim 1 wherein the unsubstituted polysaccharide is selected from the group consisting of: starch, chitosan, gums, arabinans, galactans, and mixtures thereof.**

**4. The fiber according to claim 1 wherein the unsubstituted polysaccharide comprises starch.**

**5. The fiber according to claim 1 wherein the fiber further comprises a polymer.**

**6. The fiber according to claim 5 wherein the polymer is selected from the group consisting of: polyvinyl alcohol, polyvinyl alcohol copolymers, polyvinyl alcohol derivatives, petroleum-derived polymers, polyvinyl amines and mixtures thereof.**

**7. The fiber according to claim 6 wherein the polymer comprises polyvinyl alcohol.**

**8. The fiber according to claim 1 wherein the fiber has an average fiber diameter of less than about 50  $\mu\text{m}$ .**

**9. The fiber according to claim 1 wherein the amine oxide is selected from the group consisting of: cetyltrimethylamine oxide, lauryldimethylamine oxide, cocamidopropylamine oxide and mixtures thereof.**

**10. The fiber according to claim 1 wherein the fiber exhibits a pH of less than 7.**

**11. The fiber according to claim 1 wherein the fiber as a whole exhibits no melting point.**

**12. A web comprising a fiber according to claim 1, wherein the web exhibits an initial total wet tensile greater than about 10 g/in.**

**13. A single- or multi-ply sanitary tissue product comprising a web according to claim 12.**

\* \* \* \* \*